

## UNITED STATES PATENT OFFICE

2,082,041

## PROCESS FOR PRODUCING PERMANENT MAGNETS

Clifton S. Williams, Forest Hills, Pa., assignor to Westinghouse Electric & Manufacturing Company, East Pittsburgh, Pa., a corporation of Pennsylvania

No Drawing. Application May 8, 1935,  
Serial No. 20,437

6 Claims. (Cl. 148—13)

This invention relates to a process of heat treating for improving the magnetic properties of permanent magnets.

An object of this invention is to provide for 5 improving the magnetic properties of magnetic material.

Another object of this invention is to provide a heat treatment for magnetic alloys capable of being age hardened, that will so homogenize the 10 material that its magnetic properties may be improved.

In practicing this invention, repeated cycles of similar heat treatments are provided for magnetic alloys so that the alloying elements will be dispersed throughout the alloy and the magnetic properties of the alloy may be improved.

In the preferred embodiment of this invention, the first cycle heat treatment comprises subjecting the alloys which are capable of being age 20 hardened to a temperature of from 1100° to 1350° C., and quenching from that temperature. The quenching medium may be oil, water or air. After quenching the alloy is heated to and held at a temperature of between 600° and 800° C.

This cycle of heat treatment so homogenizes the alloy that upon subjecting the homogenized alloy to a second cycle of a similar heat treatment the alloying elements will be dispersed throughout the alloy in a very finely divided form so that 25 the magnetic properties of the alloy may be improved.

In practice, the second cycle of the heat treatment is similar to the homogenizing treatment in that the alloy is subjected to a temperature of 30 between 1100° to 1350° C. and quenched. In order to set up the desired fine dispersion of the alloying elements, the quenched alloy is aged at a temperature of between 550° and 700° C. The alloys are subjected to the annealing and ageing temperatures for different periods of time depending upon the composition of the alloy treated and the size of the castings so heat treated.

This process is employed primarily to develop the magnetic properties of alloys which are capable of being age hardened such as iron cobalt alloys comprising from about 2% to 80% cobalt and from 2% to 35% of other alloying elements with the balance substantially iron. Alloys comprising iron, cobalt and either tungsten or molybdenum in which manganese may or may not be present are particularly benefited by this heat treatment.

The beneficial effect of this heat treatment is pronounced when applied to an alloy comprising 55 12% cobalt, 19% molybdenum with the balance

substantially iron. The alloy is heated at a temperature of 1300° C. for at least ten minutes and quenched in oil from that temperature. The quenched alloy is then subjected to an ageing temperature of about 700° C. for at least one-half hour and preferably from one to two hours. This cycle of heat treatment so homogenizes the alloy that when subjected to another cycle of a similar heat treatment, its magnetic properties will be fully developed.

In the second cycle of the heat treatment the homogenized alloy is reheated to a temperature of 10 1300° C. for at least ten minutes and then quenched in oil. After the quenching is effected, the alloy is aged at a temperature of 650° C. for 15 a period of from 1 to 3 hours. This cycle completes the heat treatment in that it is found that the desired precipitation or age hardening of the homogenized alloy is effected. In order that the precipitation may be closely controlled, the ageing 20 temperature of the second cycle of the heat treatment is usually lower than that of the first cycle.

When the iron, cobalt and molybdenum alloy hereinbefore identified is subjected to the heat treatment described, it is found that the magnetic properties as evidenced by the remanence 25 values of the resulting alloy, are materially increased. The development of these properties is evident from the following table showing the remanence values as determined after each of the 30 quenching and ageing treatments.

|                           | Br. (Gausses) |
|---------------------------|---------------|
| As quenched from 1300° C. | 6700          |
| As aged at 700° C.        | 8000          |
| As quenched from 1300° C. | 5100          |
| As aged at 650° C.        | 9400          |

An examination of these results shows the increase in remanence values through the application of the two cycles of heat treatment. The 40 remanence value is increased about 17% by the second cycle of heat treatment.

Although this invention has been described with reference to an iron, cobalt and molybdenum alloy, it is to be understood that it is not to be limited thereto, but is applicable to any of the permanent magnet alloys which are capable of being age hardened. Further, it is to be noted that the specific heat treatments described are capable of many modifications therein as to the 45 temperatures employed and the length of time of each of the quenching and ageing periods and that this invention is therefore not to be limited except insofar as is necessitated by the prior art and the scope of the appended claims.

I claim as my invention:

1. In the process of producing permanent magnets, in combination, quenching magnetic material from a temperature above 1100° C., ageing 5 the quenched material at a temperature of about 700° C. to homogenize it, reheating the homogenized material to a temperature above 1100° C., quenching the material, and ageing the quenched material at a temperature of about 650° 10 C. to develop its magnetic properties.
2. In the process of producing permanent magnets from age hardening alloys, in combination, quenching the alloy from a temperature above 1100° C., ageing the quenched alloy at a temperature of between 600° and 800° C. to homogenize it, reheating the homogenized alloy at a temperature above 1100° C., quenching the alloy, and ageing the alloy at a temperature of between 550° and 700° C. 15
3. In the process of producing permanent magnets from age hardening alloys, in combination, quenching the alloy from a temperature of between 1100° and 1350° C., ageing the quenched alloy at a temperature of between 600° and 800° 20 C. to homogenize it, reheating the homogenized alloy at a temperature of between 1100° and 1350° C., quenching the alloy, and ageing the alloy at a temperature of between 550° and 700° C.
4. In the process of producing permanent mag- 25

nets from age hardening alloys, in combination, quenching the alloy from a temperature of about 1300° C., ageing the quenched alloy at a temperature of about 700° C. to homogenize it, reheating the homogenized alloy at a temperature of about 1300° C., quenching the alloy, and ageing the alloy at a temperature of about 650° C. 5

5. In the process of producing permanent magnets from age hardening alloys, in combination, quenching the alloy in oil from a temperature of about 1300° C., ageing the quenched alloy at a temperature of about 700° C., reheating the alloy at a temperature of about 1300° C., quenching the alloy in oil, and ageing the alloy at a temperature of about 650° C. 10

6. In the process of producing permanent magnets from an alloy comprising about 12% cobalt, about 19% molybdenum with the balance substantially iron, in combination, heating the alloy at a temperature of between 1250° and 1350° C. 20 for at least ten minutes, quenching the alloy in oil, heating the quenched alloy at a temperature of about 700° C. for at least one-half hour, reheating the alloy at a temperature of between 1250° and 1350° C., for at least 10 minutes, quenching the reheated alloy in oil, ageing the alloy at a temperature of about 650° C. for at least one hour, and cooling the alloy to room temperature. 25

CLIFTON S. WILLIAMS.